

## UNITED STATES PATENT OFFICE

2,186,736

COUPLING COMPOUNDS FOR COLOR  
FORMING DEVELOPMENT

Wilhelm Schneider and Hans Loleit, Dessau, Germany, assignors, by mesne assignments, to Agfa Anasco Corporation, Binghamton, N. Y., a corporation of Delaware

No Drawing. Application June 24, 1938, Serial No. 215,586. In Germany July 3, 1937

12 Claims.

(Cl. 95-6)

The present invention relates to coupling compounds for color forming development.

In the process of producing photographic color pictures by the operation known as color forming development there are used developers or photographic layers containing dyestuff components which yield with the products of the oxidation of the developer a colored picture at those parts of the layer where silver has been produced. Dyestuff components which have been recommended for the purpose are phenols, naphthols, aniline, naphthylamines, amino-naphthols, and compounds having an active methylene-group, therefore compounds which contain the radical with atom grouping:



It is an object of the present invention to provide an improvement in the process of producing photographic color pictures by color forming development.

A further object of the invention resides in the provision of a new and improved class of dyestuff components, color formers or coupling compounds.

Still another object of the invention is the provision of photographic developers capable of color forming development comprising compounds from the new class of color formers.

A further object is to provide a photographic emulsion for color forming development having incorporated compounds from the new class of color formers being fast to diffusion with respect to the silver halide emulsions.

Further objects of the invention will appear from the detailed specification following herein-after.

We have found that an improvement in the process of producing photographic color pictures by color forming development may be obtained by employing as the color forming compounds capable of forming a dyestuff with the oxidation product of an aromatic amino developer, a quaternary salt of a heterocyclic base having a reactive methyl group. Suitable compounds are those of the general formula



in which  $\text{R}_1$  and  $\text{R}_2$  stand for hydrogen, inorganic or organic radicals, for example Cl, Br, I,  $\text{SO}_3\text{H}$ ,

or alkyl-, alkoxy-, aryl-, aralkyl-, amino- or substituted amino-groups, or

$\text{R}_1$  and  $\text{R}_2$  together indicate a ring system, for example a benzene ring, a naphthalene ring or a more complex ring, which ring may contain substituents;

$\text{R}_3$  stands for alkyl, aralkyl or aryl;  
 $\text{Y}$  stands for  $-\text{CH}=\text{CH}-$ , S, Se, O,



10

( $\text{R}_4$  and  $\text{R}_5$  represent alkyl, aryl or aralkyl), when  $\text{Y}=\text{CH}=\text{CH}-$ , the hydrogen atom in 4-position may be exchanged for  $\text{CH}_3$  or the hydrogen atoms in 3- and 4-positions may be exchanged for any substituents;

$\text{X}$  stands for Cl, Br, I,  $\text{SO}_3\text{H}$ ,  $\text{SO}_3\text{CH}_3$ ,  $\text{SO}_4\text{C}_2\text{H}_5$ ,  $\text{CH}_3\text{C}_6\text{H}_4\text{SO}_3$  or any other acid radical.

Suitable quaternary salts of heterocyclic bases are, for example, the salts of picoline, lutidine, quinaldine, 4-methylquinoline, 2,4-dimethylquinoline, 2-methylthiazole, 2-methyl-benzthiazole, 2,3,3-trimethyl-indolenine, and salts of these bases containing various substituents. The picolines and 2-methylthiazole yield in the development with para-dimethylamino-aniline a red picture. The bases having condensed aromatic nuclei yield a blue picture. Compounds in which a hydrogen atom of the active methyl-group is exchanged for another radical may also be used.

The dyestuff coupling components may be used both as an addition to the color developer and also to the emulsions. Since the salts of the aforesaid heterocyclic bases are easily soluble in water, no difficulty is experienced in adding them to the color developers. With color developers which contain the aforesaid substances the following colors are produced: with picoline-ethyl-iodide, with ethyl-picoline-para-toluene sulfonate, with 2,4-dimethylthiazole-dimethyl sulfate and ethyl-2,4-dimethylthiazole-para-toluene sulfonate a red picture; with quinaldine-dimethyl sulfate, with 2,4-dimethyl-quinoline-dimethyl sulfate, with  $\alpha$ -naphthoquinaldine-dimethyl sulfate, with 2-methyl-benzthiazole-dimethyl sulfate and 1,2,3,5-penta-methylindolenine-1-chloride blue pictures. When these dyestuff coupling components are mixed in the photographic layer they should be made fast to diffusion in the medium of the layer by introduction of groups, which owing to their chemical structure are capable of imparting to the dyestuff components fastness to diffusion, while retaining their solubility in water. Such groups are, for

5 instance, substantive groups as described in U. S. Patents 2,179,238 and 2,178,612 aliphatic radicals consisting of an extended saturated or unsaturated carbon chain as described in U. S. patent application Ser. No. 94,340 filed August 5, 1936, said carbon chains preferably containing radicals which impart to the finished compounds solubility in water, and further other radicals of comparatively high molecular weight, which owing to their molecular dimensions prevent diffusion of the dyestuff components within the layers or from one layer to the other, such as for instance polypeptide radicals (U. S. Patent 2,179,244), radicals of carbohydrates (U. S. patent application Ser. No. 159,518 filed August 17, 1937), radicals of natural resins (U. S. patent application Ser. No. 164,499 filed September 18, 1937), sterol radicals (U. S. patent application Ser. No. 166,832 filed October 1, 1937). Furthermore there may be used compounds in which the radical of the dyestuff component itself recurs periodically (U. S. patent application Ser. No. 171,701 filed October 29, 1937). Furthermore radicals may be introduced into the molecule of the dyestuff components which make the latter fast to diffusion, which radicals consist of hydroaromatic and hydro-heterocyclic residues, then further methane radicals (U. S. patent application Ser. No. 176,058 filed November 23, 30 1937).

Such groups may be introduced into the molecule of the dyestuff component by reaction with an amino- or carboxyl-group existing in the nucleus, an acid amide being formed. Alternatively, such groups may be linked directly with the nucleus or united in the form of a salt with the nitrogen of the heterocyclic nucleus. Dyestuff components with groups fast to diffusion are, for example, quinaldine-N-dodecyl chloride, 6-stearyl-amino-2-methyl-benzthiazole-dimethyl sulfate, bis-2-methylbenzthiazole-dimethyl sulfate of the formula



If the last named color formers are added in the usual proportion to photographic emulsions, there is obtained on development with para-dimethyl-amino-aniline a blue picture.

55 It is to be understood that the above named dyestuff components fast to diffusion are merely cited by way of example and that we do not intend to limit the scope of our invention to the specific details set forth.

60 The silver halide emulsions having dyestuff formers fast to diffusion may be made into photographic layers in the usual manner, one or more layers being on one or both sides of the carrier superimposed if necessary.

65 The layers may be used for taking black-and-white or color pictures. For the purposes of color photography several layers are with advantage sensitized for different spectral regions. If desired, several color components may be introduced into one layer and these may be so selected that on development a neutral grey picture is produced.

70

However, the emulsions may be used in another manner, for example differently sensitized emulsions having different color formers may be

distributed in the form of fine particles on a carrier.

The color picture may be produced in various ways, for example by the methods described in U. S. Patents 2,179,228, 2,179,238 and 2,178,612 and U. S. patent applications Ser. No. 94,340 filed August 5, 1936, and Ser. No. 141,093 filed May 6, 1937. Again the components located in multi-layer film may be converted into azo-dyes following development and fixing by treatment with a diazo compound such as a carbonic acid solution of tetrazotized benzidine disulfonic acid. There is thus produced in each emulsion layer together with a silver picture a dyestuff in which no structure can be perceived by magnification. The film is then treated with silver bleaching out bath, i. e. that described in British Patent 401,340 to produce the dye image. 5 10 15

In the exposed emulsion layer the picture may be produced by simple color forming development or by reversal development as described in U. S. Patent 2,179,234. Or the picture may be produced in multi-layer material, each layer containing one of said dyestuff components, by exposing the material, developing to black and white, in for instance amidol, dissolving silver from the negative so produced by bleaching in for example a chromic acid bath, forming images in the remaining silver halide, developing in a developer such as is used above, forming silver halide images by treatment in a bleaching bath, i. e., again of chromic acid, forming latent images into silver and color images in a developer capable of forming dyestuffs with said dyestuff component, removing the developed silver and fixing in thio-sulfate. In producing black-and-white pictures with the silver halide emulsion layers made by this invention, the silver may be removed or may remain in the layer together with the color picture.

What we claim is:

1. In a process of producing photographic color pictures by color forming development, the improvement which comprises developing a light-sensitive silver halide emulsion in an amino developer while causing as the color forming compound a quaternary salt of a heterocyclic base having at least one heterocyclic nucleus, said nucleus containing only one nitrogen atom and besides a methyl group linked to the carbon atom at ortho-position to said nitrogen atom to react with the oxidation products of said amino developer to form a dyestuff image. 45 50

2. In a process of producing photographic color pictures by color forming development, the improvement which comprises developing an exposed photographic silver halide emulsion with an aromatic amino developer containing as the color forming compound a quaternary salt of a heterocyclic base having at least one heterocyclic nucleus, said nucleus containing only one nitrogen atom and besides a methyl group linked to the carbon atom at ortho-position to said nitrogen atom.

3. In a process of producing photographic color pictures by color forming development, the improvement which comprises exposing a photographic silver halide emulsion containing as the color forming compound a quaternary salt of a heterocyclic base having at least one heterocyclic nucleus, said nucleus containing only one nitrogen atom and besides a methyl group linked to the carbon atom at ortho-position to said nitrogen atom and developing said emulsion with an 75

aromatic amino developer to produce a silver and dyestuff image.

4. In a process of producing photographic color pictures by color forming development, the improvement which comprises exposing a photographic silver halide emulsion containing as the color forming compound a quaternary salt of a heterocyclic base having at least one heterocyclic nucleus, said nucleus containing only one nitrogen atom and besides a methyl group linked to the carbon atom at ortho-position to said nitrogen atom.

10

5. The silver halide emulsion defined in claim 5, wherein said radicle imparting fastness to diffusion is an aliphatic carbon chain of at least 5 carbon atoms.

15

10. A silver halide emulsion defined in claim 5, wherein said heterocyclic base is selected from the class consisting of pyridines, quinolines, thiazoles and indolenines.

9. The silver halide emulsion defined in claim 5, wherein said heterocyclic base is selected from the class consisting of pyridines, quinolines, thiazoles and indolenines and wherein said radicle 15 imparting fastness to diffusion is an aliphatic carbon chain of at least 5 carbon atoms.

20

10. A silver halide gelatine emulsion for color photography containing as a color development component quinaldine-N-dodecyl-chloride.

11. A silver halide gelatine emulsion for color photography containing as a color forming development component 6-stearyl-amino-2-methylbenzthiazole-dimethyl sulfate.

25

12. A silver halide gelatine emulsion for color photography containing as a color development component bis-2-methyl - benzthiazole - dimethyl sulfate.

nucleus containing only one nitrogen atom and besides a methyl group linked to the carbon atom at ortho-position to said nitrogen atom.

7. The silver halide emulsion defined in claim 5, wherein said radicle imparting fastness to diffusion is an aliphatic carbon chain of at least 5 carbon atoms.

8. The silver halide emulsion defined in claim 5, wherein said heterocyclic base is selected from the class consisting of pyridines, quinolines, thiazoles and indolenines.

9. The silver halide emulsion defined in claim 5, wherein said heterocyclic base is selected from the class consisting of pyridines, quinolines, thiazoles and indolenines and wherein said radicle 15 imparting fastness to diffusion is an aliphatic carbon chain of at least 5 carbon atoms.

10. A silver halide gelatine emulsion for color photography containing as a color development component quinaldine-N-dodecyl-chloride.

WILHELM SCHNEIDER.

HANS LOLEIT.

20

25

30